

Oct. 23, 1951

F. A. JENKINS

2,572,156

PROCESS OF PRODUCING URANIUM HEXACHLORIDE

Filed July 13, 1943



INVENTOR.

Francis A. Jenkins

BY

Robert A. Danenber

ATTORNEY.

## UNITED STATES PATENT OFFICE

2,572,156

PROCESSES OF PRODUCING URANIUM  
HEXACHLORIDEFrancis A. Jenkins, Berkeley, Calif., assignor to  
the United States of America as represented by  
the United States Atomic Energy Commission

Application July 13, 1943, Serial No. 494,447

7 Claims. (Cl. 23—14.5)

1

The present invention relates to  $UCl_6$  and processes of producing the same.

Heretofore the compound  $UCl_6$  has not been known. Moreover, it has been predicted that the possibility of its production is virtually negligible in view of its expected great instability. This view is entirely plausible since the tetrahalides of uranium form a series decreasing in stability in a regular manner from the fluoride through the chloride and the bromide to the iodide, and since  $UF_6$  is extremely unstable. Thus it has always been assumed that the hexahalide series of uranium terminates abruptly at the compound  $UF_6$ .

The present invention is predicated upon the discoveries that uranium pentachloride is a binary compound of the form  $UCl_4 \cdot UCl_6$  rather than a monomeric compound of the form  $UCl_5$  and that in this compound the molecular bond may be broken under certain conditions, producing as two independent compounds  $UCl_4$  and  $UCl_6$ .

Accordingly, it is an object of the invention to provide  $UCl_6$  as a stable compound.

Another object of the invention is to provide a process of producing  $UCl_6$  as a stable compound.

Another object of the invention is to provide a process of producing  $UCl_6$  which utilizes uranium pentachloride.

Another object of the invention is to provide a process utilizing uranium pentachloride, whereby  $UCl_4$  and  $UCl_6$  are produced and separated.

A further object of the invention is to provide a process in which the molecular bond in the binary compound  $UCl_4 \cdot UCl_6$  is broken, whereby  $UCl_4$  and  $UCl_6$  are produced as independent compounds.

A further object of the invention is to provide a process utilizing  $UCl_4 \cdot UCl_6$ , whereby  $UCl_4$  and  $UCl_6$  are produced and  $UCl_6$  is sublimed away from  $UCl_4$ .

A still further object of the invention is to provide a combination heating and vacuum process of producing  $UCl_4$  and  $UCl_6$  from uranium pentachloride and of separating these products from each other.

The invention, both as to its organization and method of operation, together with further objects and advantages thereof, will best be understood by reference to the following specification taken in connection with the accompanying drawing, in which the single figure is a schematic illustration of apparatus suitable for carrying out the processes of the present invention.

In accordance with the present invention, a

2

suitable charge of uranium pentachloride is placed in a substantially conventional molecular still which comprises a hot surface heated in any suitable manner, such, for example, as by a hot sand bath, and a cold surface cooled in any suitable manner, such, for example, as by liquid air. In the still the hot surface and the cold surface are disposed in spaced apart relation, and the space therebetween is evacuated to an extremely low pressure by suitable vacuum pumping apparatus. More particularly, the charge is placed on the hot surface of the still and the temperature of the sand bath is suitably controlled, in order that the charge is maintained at a temperature within the range 80° to 180° C. Also, the amount of liquid air which is applied to the cold surface of the still is such that the temperature of the cold surface is maintained at 10° C. or below. Finally, the vacuum pumping apparatus is adjusted, so that the pressure within the still between the hot surface and the cold surface is maintained at a value between  $10^{-6}$  and  $10^{-3}$  mm. Hg. Preferably in carrying out the process, the space between the normal hot surface and the normal cold surface of the still is evacuated to obtain the subatmospheric pressure within the range mentioned, before the normal hot surface is heated by the sand bath and the normal cold surface is cooled by the liquid air.

When the charge of uranium pentachloride is thus heated under subatmospheric pressure, it is converted into  $UCl_4$  and  $UCl_6$ , the  $UCl_6$  being sublimed as it is produced. The  $UCl_4$  remains as a residue upon the hot surface and the sublimed  $UCl_6$  traverses the space between the hot and cold surfaces to condense upon the cold surface in the form of iridescent, dark green, fine-grained crystals as the temperature of the charge is above the sublimation point of  $UCl_6$  and below the sublimation point of  $UCl_4$ .

The process is continued until the charge of uranium pentachloride is substantially completely converted, at which time the residue remaining on the hot surface is substantially chemically pure  $UCl_4$  and the sublimate collected on the cold surface is substantially pure  $UCl_6$ . At this time, when further production and sublimation of  $UCl_6$  ceases and the process is complete, the  $UCl_4$  residue is removed from the hot surface and the  $UCl_6$  sublimate is removed from the cold surface. Ordinarily in carrying out the process a charge of 100 grams of uranium pentachloride may be substantially completely converted into a residue of  $UCl_4$  and a sublimate of  $UCl_6$  in approximately three hours.

It is virtually essential that the still be transferred to a dry cabinet containing  $\text{CO}_2$  or other inert gas before it is opened, in view of the fact that the sublimate  $\text{UCl}_6$  is extremely hygroscopic and readily decomposes in the presence of ordinary atmosphere into  $\text{UO}_2\text{Cl}_2$ . The product  $\text{UCl}_6$  is then bottled in an atmosphere of  $\text{CO}_2$  or in a vacuum and sealed for future use. The product  $\text{UCl}_6$  so produced is particularly well suited for use in vacuum apparatus, in that it has a very much greater vapor pressure at a considerably lower temperature than other volatile chlorides of uranium, such, for example, as  $\text{UCl}_4$ .

While the process may be carried out at a temperature below the lower end of the preferred range, it is noted that in the event the temperature is much lower than  $80^\circ \text{C}$ . the yield of  $\text{UCl}_6$  from the charge is extremely poor and very slow. Similarly, while the process may be carried out at a temperature above the upper end of the preferred range, it is noted that in the event the temperature is much higher than  $180^\circ \text{C}$ . the  $\text{UCl}_4$  produced as a residue in the charge itself begins to sublime, and the  $\text{UCl}_6$  is decomposed to  $\text{UCl}_4$  and  $\text{Cl}_2$  before it can be sublimed from the hot surface. In other words, it is essential that the process be carried out under conditions such that the newly formed  $\text{UCl}_6$  is removed from the hot zone, or region of maximum temperature, before any substantial decomposition of the product  $\text{UCl}_6$  can take place. Also, when the temperature is much higher than  $180^\circ \text{C}$ . the sublimate is of very low chemical purity in that large amounts of  $\text{UCl}_4$  are mixed with the  $\text{UCl}_6$ , and furthermore the yield is low.

Of course the vapor pressure-temperature curves of  $\text{UCl}_6$  and  $\text{UCl}_4$  are of usual form, the vapor pressure increasing disproportionately with temperature, whereby there is a negligible sublimation of  $\text{UCl}_4$  within the normal sublimation temperature range of  $\text{UCl}_6$ . However, for practical purposes of obtaining correspondingly reasonable yields, it may be said that the sublimation temperature of  $\text{UCl}_6$  is well below that of  $\text{UCl}_4$  as indicated below:

| Temperature, $^\circ\text{C}$ | Vapor Pressure<br>mm. Hg |                  |
|-------------------------------|--------------------------|------------------|
|                               | $\text{UCl}_6$           | $\text{UCl}_4$   |
| 0                             | 0.005                    | ( <sup>2</sup> ) |
| 20                            | 0.023                    |                  |
| 40                            | 0.08                     |                  |
| 60                            | 0.22                     |                  |
| 80                            | 0.59                     |                  |
| 100                           | 1.35                     |                  |
| 120                           | 2.95                     |                  |
| 140                           | 5.75                     |                  |
| 160                           | 11.07                    |                  |
| 180                           | 18.60                    |                  |
| 200                           | 32.35                    |                  |
| 250                           |                          | ( <sup>1</sup> ) |
| 300                           |                          |                  |
| 350                           | 0.0006                   |                  |
| 400                           | 0.0048                   |                  |
| 450                           |                          | 0.050            |
| 500                           |                          | 0.70             |
| 550                           |                          | 5.5              |
| 600                           |                          | 15.0             |

<sup>1</sup> Decomposition of  $\text{UCl}_6$  begins.

<sup>2</sup> Pressure of  $\text{UCl}_4$  below  $300^\circ \text{C}$ . is negligible.

#### Examples

When the process is carried out employing a charge of uranium pentachloride,  $\text{UCl}_4 \cdot \text{UCl}_6$ , it is believed that the molecular bond is broken, whereby  $\text{UCl}_4$  and  $\text{UCl}_6$  are produced as independent monomeric compounds, and that the  $\text{UCl}_6$  is sublimed away from the  $\text{UCl}_4$ , as it is noted that the sublimation temperature of  $\text{UCl}_6$

is considerably below that of  $\text{UCl}_4$  and that  $\text{UCl}_6$  has a much higher vapor pressure at a given temperature than  $\text{UCl}_4$ . Further, it is thought that the following specific reaction takes place:



Theoretically, one mole of the binary compound  $\text{UCl}_4 \cdot \text{UCl}_6$  (831 grams) should yield one mole of the monomeric compound  $\text{UCl}_4$  (380 grams) and one mole of the monomeric compound  $\text{UCl}_6$  (451 grams); the weight percent of chlorine in the residue  $\text{UCl}_4$  should be 37.34; and the weight percent of chlorine in the sublimate  $\text{UCl}_6$  should be 47.19. The analyses of the residue and the sublimate produced incident to carrying out the present process checked very closely with the theoretical values indicated. For instance, in a typical run utilizing a charge of 100 grams of uranium pentachloride, when the process is substantially complete analyses have indicated a weight of  $\text{UCl}_4$  residue of 47 grams, a weight of  $\text{UCl}_6$  sublimate collected of 52 grams, and a weight of  $\text{UCl}_6$  sublimate lost of one gram. Also, analyses for total uranium and total chlorine, made gravimetrically by tested procedure, indicated the following for the sublimed material:

|                   | Per cent |
|-------------------|----------|
| Total U           | 53.30    |
| Quadrivalent U    | (2.31)   |
| Chlorine          | 46.41    |
|                   | 99.71    |
| Atomic ratio Cl/U | 5.85     |

When allowance is made for the inevitable decomposition which accompanies any transfer of material, except under vacuum in thoroughly baked-out apparatus, the analyses are so close to that required for  $\text{UCl}_6$  that there can be no serious doubt that the sublimate is substantially chemically pure  $\text{UCl}_6$ ; the atomic ratio Cl/U of 5.85 obtained from the analyses is well within experimental error of the theoretical atomic ratio Cl/U of 6. Also, analyses of the residue yield an atomic ratio of Cl/U of 3.94, clearly indicating that the residue is substantially chemically pure  $\text{UCl}_4$ .

In further evidence of the fact that the binary compound uranium pentachloride is converted into the two monomeric compounds mentioned, it is pointed out that check runs in the still under the conditions specified, utilizing the residue  $\text{UCl}_4$  and the sublimate  $\text{UCl}_6$ , yield very interesting results. More particularly, in a check run utilizing the residue  $\text{UCl}_4$ , there is virtually no sublimate, indicating that the residue is already substantially chemically pure  $\text{UCl}_4$ . On the other hand, in a check run utilizing the sublimate  $\text{UCl}_6$ , there is virtually no residue, indicating that the sublimate is already substantially chemically pure  $\text{UCl}_6$ .

Preferably, the uranium pentachloride employed as a charge in the still in carrying out the present process is produced by the improved process disclosed in the copending application of Horace R. McCombie, Serial No. 506,336, filed October 15, 1943. More particularly, it has been found that when the charge of uranium pentachloride is produced in accordance with the process disclosed in the above mentioned McCombie application as contrasted with other known processes, the yield of  $\text{UCl}_6$  from the charge in the still is considerably higher, and of the order of 50% greater.

Referring now more particularly to the single

figure of the drawing, there is illustrated a substantially conventional molecular still which is suitable for carrying out the present process, the still comprising lower and upper casing members 11 and 12, respectively, formed of Pyrex glass. The lower casing member 11 is provided with an outwardly directed sealing flange 13 adjacent the upper end thereof, and the upper casing member 12 is provided with an outwardly directed sealing flange 14 adjacent the lower end thereof, the sealing flanges 13 and 14 being adapted to mate to provide a hermetic seal between the lower and upper casing members 11 and 12, respectively, of the still. The upper casing member 12 is provided with a re-entrant portion 15 projecting into and spaced inwardly from the side wall of the lower casing member 11, in order to define a vacuum space between the lower and upper casing members 11 and 12, respectively. The lower casing member 11 is provided with a bottom end wall 16, constituting a normally hot surface adapted to receive a charge 17 of uranium pentachloride; and the re-entrant portion 15 of the upper casing member 12 is provided with a bottom end wall 18 constituting a normally cold surface. The bottom end wall 16 of the lower casing member 11 is arranged within a hot sand bath 19, whereby the charge 17 is heated; and the re-entrant portion 15 of the upper casing member 12 is adapted to contain a body 20 of liquid air, whereby the surface 18 is cooled. Finally, the lower casing member 11 has a conduit 21 formed integrally therewith and communicating with the vacuum space disposed between the lower and upper casing members 11 and 12. The conduit 21 is suitably connected to vacuum pumping apparatus, not shown, and includes a stopcock 22.

In the operation of the molecular still, the charge 17 of uranium pentachloride is first positioned on the normally heated surface 16 of the lower casing member 11, the upper casing member 12 is brought into relation, and the flanges 13 and 14 are appropriately sealed. The pumping apparatus is started, and the stopcock 22 is opened, whereby the pressure in the vacuum space between the lower casing member 11 and the upper casing member 12 is lowered to a pressure of the order of  $10^{-6}$  to  $10^{-3}$  mm. Hg. The temperature of the sand bath 19 is suitably adjusted, whereby the temperature of the charge 17 is maintained within the range 80° to 180° C., and the body 20 of liquid air is poured into the re-entrant portion 15 of the upper casing member 12, whereby the cold surface 18 is suitably cooled to a temperature of the order of 10° C. or below. When the charge 17 is thus heated, the conversion takes place, whereby the charge 17 of uranium pentachloride is progressively converted into  $\text{UCl}_4$  and  $\text{UCl}_6$ , the  $\text{UCl}_6$  subliming as it is produced and traversing the space between the hot surface 16 and the cold surface 18. The  $\text{UCl}_4$  remains as a residue upon the hot surface 16, and the sublimate  $\text{UCl}_6$  is condensed to its solid state upon the cold surface 18. After the process has been completed, the stopcock 22 is closed and the still is removed to the dry cabinet and opened, as previously explained. It will be noted from the foregoing that, since the  $\text{UCl}_6$  is sublimed or vaporized substantially as it is produced [apparently by the disruption of the molecular bond of the uranium pentachloride ( $\text{UCl}_4\text{UCl}_6$ )] it is not permitted to remain in the hot zone for a time sufficient to cause any substantial degree of thermal decomposition

thereof, thus insuring maximum production and recovery of  $\text{UCl}_6$  as such.

Reconsidering the properties of the monomeric compound  $\text{UCl}_6$ , it is again noted that this product is of fine crystalline structure, having an iridescent dark green color. The vapor pressure of the product  $\text{UCl}_6$  is of the order of 1 to 3 mm. Hg at 100° C.; and the product is extremely hygroscopic and unstable in ordinary atmosphere. When the product  $\text{UCl}_6$  is subjected to normal atmosphere containing moisture, it rapidly decomposes to  $\text{UO}_2\text{Cl}_2$ . However, the product  $\text{UCl}_6$  exists in stable form in dry air, nitrogen, helium, and other inert gases.

The vapor of  $\text{UCl}_6$  readily attacks most of the ordinary metals considerably more actively than does the vapor of  $\text{UCl}_4$ , decomposing to  $\text{UCl}_4$ . For example,  $\text{UCl}_6$  vapor at 100° C. readily attacks copper, copper alloys, silver, iron, graphite, etc., and exhibits no substantial attack upon stainless steel, monel metal, nickel, and gold. The product  $\text{UCl}_6$  is soluble in water, decomposing immediately to  $\text{UO}_2\text{Cl}_2$ , and cannot be dissolved in ionic oxygenated solvents without decomposition to  $\text{UO}_2\text{Cl}_2$ . Finally, the product  $\text{UCl}_6$  is readily soluble in  $\text{CCl}_4$ , producing a dark brown solution.

While there has been described what is at present considered to be the preferred embodiment of the invention, it will be understood that various modifications may be made therein and it is intended to cover in the appended claims all such modifications as fall within the true spirit and scope of the invention.

What is claimed is:

1. The process comprising heating uranium pentachloride to a temperature which is sufficiently high to convert it to  $\text{UCl}_4$  and  $\text{UCl}_6$  and which is above the sublimation temperature of  $\text{UCl}_6$  and below the sublimation temperature of  $\text{UCl}_4$ , said heating being conducted under conditions such that the  $\text{UCl}_6$  which is produced is sublimed as it is formed, and recovering the  $\text{UCl}_6$  thus produced.

2. The process comprising heating uranium pentachloride to a temperature which is sufficiently high to convert it to  $\text{UCl}_4$  and  $\text{UCl}_6$  and which is above the sublimation temperature of  $\text{UCl}_6$  and below the sublimation temperature of  $\text{UCl}_4$  and simultaneously subjecting it to a pressure not appreciably greater than  $10^{-3}$  mm. Hg, said heating being conducted under conditions such that the  $\text{UCl}_6$  which is produced is sublimed as it is formed, and recovering the  $\text{UCl}_6$  thus produced.

3. The process comprising heating uranium pentachloride to a temperature within the range 80° to 180° C. and simultaneously subjecting it to a pressure not appreciably greater than  $10^{-3}$  mm. Hg, whereby  $\text{UCl}_6$  is produced and sublimed substantially as it is formed, and recovering the  $\text{UCl}_6$  thus produced.

4. The process comprising heating  $\text{UCl}_4\text{UCl}_6$  to an elevated temperature and simultaneously subjecting it to a subatmospheric pressure, whereby  $\text{UCl}_4$  and  $\text{UCl}_6$  are produced, subliming the  $\text{UCl}_6$  away from the  $\text{UCl}_4$  under conditions such that the  $\text{UCl}_6$  is removed from the heated zone before any substantial decomposition thereof takes place, and recovering the  $\text{UCl}_6$  thus produced.

5. The process comprising heating  $\text{UCl}_4\text{UCl}_6$  to an elevated temperature and simultaneously subjecting it to a subatmospheric pressure, whereby  $\text{UCl}_4$  and  $\text{UCl}_6$  are produced, subliming

the  $\text{UCl}_6$  away from the  $\text{UCl}_4$ , and condensing the sublimed  $\text{UCl}_6$  to its solid state; the  $\text{UCl}_6$  being removed from the heated zone as it is formed and before any substantial decomposition thereof takes place, and recovering the  $\text{UCl}_6$  thus produced.

6. The process comprising subjecting



simultaneously to heat and a subatmospheric pressure in a heated zone, whereby  $\text{UCl}_4$  and  $\text{UCl}_6$  are produced, subliming the  $\text{UCl}_6$  as it is produced, conducting the sublimed  $\text{UCl}_6$  away from the heated zone to a remotely disposed cooled zone, condensing the sublimed  $\text{UCl}_6$  to its solid state in the cooled zone, and recovery the  $\text{UCl}_6$  thus produced.

7. The process comprising converting uranium pentachloride to  $\text{UCl}_4$  and  $\text{UCl}_6$  by heating it to

a temperature within the range 80° to 180° C. while subjecting it to a pressure not appreciably greater than  $10^{-3}$  mm. Hg, subliming the  $\text{UCl}_6$ , conducting the sublimed  $\text{UCl}_6$  substantially as it is formed away from the  $\text{UCl}_4$  to a remotely disposed cooled zone, and condensing the sublimed  $\text{UCl}_6$  to its solid state in the cooled zone.

F. A. JENKINS.

#### REFERENCES CITED

The following references are of record in the file of this patent:

Chemical Abstracts, vol. V, 1911, page 3772, Otto Ruff and Alfred Heinzelmann, Danzig Z. Anorg. Chem. 72, pages 63-84.

Mellor, "Comprehensive Treatise on Inorganic and Theoretical Chemistry, vol. XII, 1932, pages 35, 83, and 84. (Copy in Division 59.)